# EUROPEAN PATENT SPECIFICATION

(11) **EP 3 419 828 B1**
(45) Date of publication and mention of the grant of the patent: **18.12.2019**
(21) Application number: 17705625.6
(22) Date of filing: 17.02.2017
(51) Int. Cl.: B41F 30/04, B41F 13/193, B41N 10/04

(54) **RUBBER BLANKET FOR A PRINTING CYLINDER OF A PRINTING MACHINE**
GUMMITUCH FÜR EINEN DRUCKZYLINDER EINER DRUCKMASCHINE
BLANCHET DE CAOUTCHOUC POUR UN CYLINDRE D'IMPRESSION D'UNE MACHINE D'IMPRESSION

(30) Priority: 22.02.2016 IT UB20160940
(43) Date of publication of application: 02.01.2019
(73) Proprietor: Trelleborg Coated Systems Italy S.p.A., 20124 Milano (IT)
(72) Inventor: HERTZOG, Denis, 68500 Berrwiller (France) (FR); HARAUX, Sophie, 68700 Aspach-Michelbach (France) (FR); TOMBOLATO, Fabio, 36020 Pove del Grappa (Vicenza) (IT)
(74) Representative: Rapisardi, Mariacristina
(86) International application number: PCT/EP2017/053599
(87) International publication number: WO 2017/144358

(56) References cited:
- EP-A1- 2 502 753
- WO-A1-2009/010123
- WO-A1-2015/074908
- US-A1- 2003 116 044
- US-A1- 2003 124 926

## Description

The present invention relates to rubber blankets for printing cylinders of offset printing machines, especially, but not exclusively, of the sheet-fed offset type.

As is well known to the person skilled in the art, in these printing machines, mounted on a printing cylinder made of metal and rotating about its own axis, there is a multilayer product, known in the industry as a printing rubber blanket, which covers the outer surface of the printing cylinder.

A printing rubber blanket has an upper elastomeric layer that acts as a printing surface, a compressible intermediate layer, and one or more lower reinforcement layers made of fabric, the last of which is applied on the surface of the printing cylinder.

This type of printing rubber blanket exhibits some drawbacks.

Firstly, in order to be correctly fixed to the cylinder, the last lower layer requires the application of a special adhesive layer, which, though on the one hand it achieves its purpose, on the other hand it complicates the replacement of the rubber blanket, imposing machine downtimes, even long ones, with consequent negative repercussions on productivity.

Secondly, a rubber blanket with such a structure does not easily lend itself to grinding to bring the overall thickness to the desired value.

In particular, in order to bring the overall thickness of the rubber blanket to the desired value, it is sometimes necessary to grind the upper layer, which, however, for the purpose of optimizing printing quality has a mirror-like surface finish which must be restored.

EP2502753 A1 discloses a printing blanket according to the preamble of claim 1 made of layers detachably connected to each other.

Therefore, the task of the present invention is to provide a printing rubber blanket capable of overcoming the drawbacks found in the prior art.

In particular, one object of the present invention is to provide a rubber blanket for a printing cylinder having a structure that makes it adaptable in a versatile manner to production in various thicknesses and to a simplified mounting on and removal from the printing cylinder.

Another object of the present invention is to provide a rubber blanket for a printing cylinder which offers the desired mechanical properties with a substantial reduction in costs.

These objects are achieved, according to the present invention, by virtue of a rubber blanket for a printing cylinder of a printing machine as defined in claim 1.

Further preferred embodiments of the invention are defined in the dependent claims.

Advantageously, said expanded elastomeric material has a porosity adapted so as to impart to the lower layer a susceptibility to abrasion for grinding the thickness of said lower layer.

Advantageously, said expanded elastomeric material also has a porosity adapted so as to impart to the lower layer a susceptibility to direct adhesion to said cylinder without the addition of another adhesive layer.

Said layers of said rubber blanket are undetachably connected to each other.

According to the invention, said expanded elastomeric material is a thermoplastic elastomer, comprising a thermoplastic polyurethanene, or a vulcanized thermoset elastomer, said vulcanized thermoset elastomer comprising at least one selected from among PU, NBR, EPDM, SBR and EPM.

These and other aspects will become more evident from the description that follows of preferred embodiments of the invention, which must be considered as non-limiting examples.

The description makes reference to the appended drawings, in which:
- Fig. 1 shows a cross-section of a printing rubber blanket according to a first preferred embodiment of the present invention;
- Fig. 2 shows a cross-section of a printing rubber blanket according to a second preferred embodiment of the present invention;
- Fig. 3 shows a cross-section of a printing rubber blanket according to a third preferred embodiment of the present invention;
- Fig. 4 shows the rubber blanket of figure 3 mounted on a printing cylinder.

The printing rubber blanket for a printing cylinder of a printing machine is generally indicated by the reference number 1.

The printing rubber blanket 1 has a multilayer structure comprising at least a lower layer 2 having a contact surface 2a in contact with the printing cylinder 8, at least an upper printing layer 3, 3', and at least an intermediate fabric reinforcement layer 4 interposed between the upper layer 3, 3' and the lower layer 2.

The lower layer 2 is made of expanded elastomeric material.

Advantageously, the expanded elastomeric material has a porosity adapted so as to impart to the lower layer 2 a susceptibility to abrasion for grinding the thickness of the lower layer 2.

Advantageously, moreover, the expanded elastomeric material has a porosity adapted so as to impart to the lower layer 2 a susceptibility to direct adhesion to the printing cylinder without the addition of another adhesive layer.

The elastomeric material is expanded with microspheres or expanding agents such as azodicarbonamide.

The expanded elastomeric material can be a thermoplastic elastomer or a vulcanized thermoset elastomer.

The expanded elastomeric material, if thermoplastic, comprises a thermoplastic polyurethane.

The expanded elastomeric material, if thermoset, comprises a vulcanized rubber comprising at least one polymer selected from among PU (polyurethane rubber), NBR (nitrile butadiene rubber), EPDM (ethylene propylene diene monomer rubber), SBR (styrene butadiene rubber) and EPM (ethylene propylene rubber).

Preferably, the compact elastomeric material forming the upper layer 3, 3' can also be, in general, a thermoplastic or thermoset elastomer.

Preferably, the upper layer 3, 3' is produced by deposition of a thermoplastic polyurethane elastomer by casting so as to impart adequate smoothness and a mirror finish to the printing surface 3a.

The fabric reinforcement layer 4 is preferably made of cotton fibres or a blend of cotton and polyester fibres.

With reference to figure 1, the rubber blanket 1 consists of a series of two upper layers 3, 3' each having a uniform thickness of 0.35 mm, a lower layer 2 having a uniform thickness of 0.50 mm, an intermediate fabric reinforcement layer 4 having a uniform thickness of 0.45 mm, a first adhesive layer 5 for fixing the intermediate layer 4 to the upper layer 3, and a second adhesive layer 6 for fixing the intermediate layer 4 to the lower layer 2.

With reference to figure 2, the rubber blanket 1 consists of an upper layer 3 having a uniform thickness of 0.35 mm, a lower layer 2 having a uniform thickness of 0.50 mm, an intermediate fabric reinforcement layer 4 having a uniform thickness of 0.45 mm, a first adhesive layer 5 for fixing the intermediate layer 4 to the upper layer 3, and a second adhesive layer 6 for fixing the intermediate layer 4 to the lower layer 2.

With reference to figure 3, the rubber blanket 1 consists of an upper layer 3 having a uniform thickness of 0.55 mm, a lower layer 2 having a uniform thickness of 0.30 mm, an intermediate fabric reinforcement layer 4 having a uniform thickness of 0.45 mm, a first adhesive layer 5 for fixing the intermediate layer 4 to the upper layer 3, and a second adhesive layer 6 for fixing the intermediate layer 4 to the lower layer 2.

The lower expanded elastomeric layer 2 of the rubber blanket 1 employed in the above-described solutions has the mechanical characteristics shown in the following table.

| blanket | thickness (mm) | Compressibility: deformation at 1.20MPa (µm) | Load at 150µm (MPa) | Pore diameter (µm) |
|---|---|---|---|---|
| Fig. 1 and 2 | 0.5 | 105 | 2.08 | 40-100 |
| Fig. 3 | 0.3 | 91 | 2.93 | 40-120 |

Where the compressibility test measures the deformation by compression of the layer subjected to a fixed pressure (normal force per surface unit), whilst the load test measures the load that is necessary (normal force per surface unit) to obtain a fixed deformation (150 microns) under compression.

The invention uses a lower layer 2 having a deformation at 120 MPa comprised between 80 and 120 microns and a load comprised between 2 and 3 MPa to obtain a deformation of 150 microns.

A rubber blanket with the above-described structure, due to the fact that it comprises a lower layer made of an expanded elastomeric material with an adapted porosity, enables both a high grip to be obtained on the printing cylinder without using adhesives and grinding to be performed to bring the overall thickness of the rubber blanket to the desired value by abrasion of the contact surface of the lower layer without touching the printing surface of the upper layer which has the mirror finish.

The printing rubber blanket thus conceived is susceptible to various modifications and variants, all falling within the scope of the invention; moreover, all of the details can be replaced with other technically equivalent elements. In practice, the materials used, as well as the dimensions, can vary according to requirements and the state of the art.

## Claims

1. A rubber blanket (1) for a printing cylinder (8) of a printing machine,
comprising at least an upper printing layer (3, 3') made of compact elastomeric material, at least a lower layer (2) having a contact surface (2a) in contact with said printing cylinder (8), and at least one fabric reinforcement layer (4) interposed between the upper layer (3) and the lower layer (2), wherein said lower layer (2) is made of expanded elastomeric material, **characterized in that** said lower layer (2) has a deformation at 120 MPa comprised between 80 micron and 120 micron and a load comprised between 2 MPa and 3 MPa to obtain a deformation of 150 micron, said expanded elastomeric material being a thermoplastic elastomer comprising a thermoplastic polyurethane or being a vulcanized thermoset elastomer, said vulcanized thermoset elastomer comprising at least one selected from PU, NBR, EPDM, SBR and EPM.

2. The rubber blanket (1) according to claim 1, **characterized in that** said layers (3, 3'; 2; 4) are permanently connected to each other.

3. The rubber blanket (1) according to claim 1, **characterized in that** it comprises a sole fabric reinforcement layer (4), a first adhesive layer (5) for fixing said intermediate layer (4) to said upper layer (3), and a second adhesive layer (6) for fixing said intermediate layer (4) to said lower layer (2).

4. The rubber blanket (1) according to claim 1, **characterized in that** said intermediate layer (4) is at least partially formed from cotton fabric.

5. The rubber blanket (1) according to claim 1, **characterized in that** it consists of an intermediate fabric reinforcement layer (4) having a thickness of 0.45 mm, a first adhesive layer (5) for fixing said intermediate layer (4) to said upper layer (3, 3'), a second adhesive layer (6) for fixing said intermediate layer (4) to said lower layer (2), a lower layer (2) having a thickness of 0.50 mm, and a series of two upper layers (3, 3') each having a thickness of 0.35 mm.

6. The rubber blanket (1) according to claim 1, **characterized in that** it consists of an intermediate fabric reinforcement layer (4) having a thickness of 0.45 mm, a first adhesive layer (5) for fixing said intermediate layer (4) to said upper layer (3), a second adhesive layer (6) for fixing said intermediate layer (4) to said lower layer (2), a lower layer (2) having a thickness of 0.50 mm, and an upper layer (3) having a thickness of 0.35 mm.

7. The rubber blanket (1) according to claim 1, **characterized in that** it consists of an intermediate fabric reinforcement layer (4) having a thickness of 0.45 mm, a first adhesive layer (5) for fixing said intermediate layer (4) to said upper layer (3), a second adhesive layer (6) for fixing said intermediate layer (4) to said lower layer (2), a lower layer (2) having a thickness of 0.30 mm, and an upper layer (3) having a thickness of 0.55 mm.

8. A printing cylinder (8) on which the rubber blanket (1) according to any preceding claim is mounted, said contact surface (2a) of said lower layer (2) being directly in contact with said cylinder (8) without any interposition of adhesive.

## Patentansprüche

1. Gummituch (1) für einen Druckzylinder einer Druckmaschine,
umfassend mindestens eine obere Druckschicht (3, 3') aus kompaktem Elastomermaterial, mindestens eine untere Schicht (2) mit einer Kontaktfläche (2a) in Kontakt mit dem Druckzylinder (8) und mindestens eine Gewebeverstärkungsschicht (4), die zwischen der oberen Schicht (3) und der unteren Schicht (2) angeordnet ist, wobei die untere Schicht (2) aus expandiertem Elastomermaterial besteht, **dadurch gekennzeichnet, dass** die untere Schicht (2) eine Verformung bei 120 MPa zwischen 80 Mikron und 120 Mikron und eine Last zwischen 2 MPa und 3 MPa aufweist, um eine Verformung von 150 Mikron zu erhalten, wobei das expandierte Elastomermaterial ein thermoplastisches Elastomer ist, das ein thermoplastisches Polyurethan umfasst, oder ein vulkanisiertes wärmehärtbares Elastomer ist, wobei das vulkanisierte wärmehärtbare Elastomer mindestens eines ausgewählt aus PU, NBR, EPDM, SBR und EPM umfasst.

2. Gummituch (1) nach Anspruch 1, **dadurch gekennzeichnet, dass** die Schichten (3, 3'; 2; 4) dauerhaft miteinander verbunden sind.

3. Gummituch (1) nach Anspruch 1, **dadurch gekennzeichnet, dass** es eine Sohlengewebeverstärkungsschicht (4), eine erste Klebeschicht (5) zum Befestigen der Zwischenschicht (4) an der oberen Schicht (3) und eine zweite Klebeschicht (6) zum Befestigen der Zwischenschicht (4) an der unteren Schicht (2) umfasst.

4. Gummituch (1) nach Anspruch 1, **dadurch gekennzeichnet, dass** die Zwischenschicht (4) mindestens teilweise aus Baumwollgewebe gebildet ist.

5. Gummituch (1) nach Anspruch 1, **dadurch gekennzeichnet, dass** es aus einer Zwischengewebeverstärkungsschicht (4) mit einer Dicke von 0,45 mm und einer ersten Klebeschicht (5) zum Befestigen der Zwischenschicht (4) an der oberen Schicht besteht (3, 3'), einer zweiten Klebeschicht (6) zum Befestigen der Zwischenschicht (4) an der unteren Schicht (2), einer unteren Schicht (2) mit einer Dicke von 0,50 mm und einer Reihe von zwei oberen Schichten (3, 3') mit einer Dicke von jeweils 0,35 mm besteht.

6. Gummituch (1) nach Anspruch 1, **dadurch gekennzeichnet, dass** es aus einer Zwischengewebeverstärkungsschicht (4) mit einer Dicke von 0,45 mm und einer ersten Klebeschicht (5) zum Befestigen der Zwischenschicht (4) an der oberen Schicht besteht (3), einer zweiten Klebeschicht (6) zum Befestigen der Zwischenschicht (4) an der unteren Schicht (2), einer unteren Schicht (2) mit einer Dicke von 0,50 mm und einer oberen Schicht (3) mit einer Dicke von 0,35 mm besteht.

7. Gummituch (1) nach Anspruch 1, **dadurch gekennzeichnet, dass** es aus einer Zwischengewebeverstärkungsschicht (4) mit einer Dicke von 0,45 mm, einer ersten Klebeschicht (5) zum Befestigen der Zwischenschicht (4) an der oberen Schicht besteht (3), einer zweiten Klebeschicht (6) zum Befestigen der Zwischenschicht (4) an der unteren Schicht (2), einer unteren Schicht (2) mit einer Dicke von 0,30 mm und einer oberen Schicht (3) mit einer Dicke von 0,55 mm besteht.

8. Druckzylinder (8), auf dem das Gummituch (1) nach einem der vorhergehenden Ansprüche montiert ist, wobei die Kontaktfläche (2a) der unteren Schicht (2) ohne jegliche Klebstoffzwischenlage in direktem Kontakt mit dem Zylinder (8) steht.

## Revendications

1. Blanchet de caoutchouc (1) pour un cylindre d'impression (8) d'une machine d'impression,
comprenant au moins une couche d'impression (3, 3') supérieure constituée d'un matériau élastomère compact, au moins une couche inférieure (2) comportant une surface de contact (2a) en contact avec ledit cylindre d'impression (8), et au moins une couche de renforcement (4) en tissu interposée entre la couche supérieure (3) et la couche inférieure (2), dans lequel ladite couche inférieure (2) est constituée d'un matériau élastomère expansé, **caractérisé en ce que** ladite couche inférieure (2) comporte une déformation à 120 MPa comprise entre 80 et 120 microns et une charge comprise entre 2 et 3 MPa pour obtenir une déformation de 150 microns, ledit matériau élastomère expansé étant un élastomère thermoplastique comprenant un polyuréthane thermoplastique ou étant un élastomère thermodurci vulcanisé, ledit élastomère thermodurci vulcanisé comprenant au moins un élément sélectionné parmi PU, NBR, EPDM, SBR et EPM.

2. Blanchet de caoutchouc (1) selon la revendication 1, **caractérisé en ce que** lesdites couches (3, 3' ; 2 ; 4) sont reliées en permanence l'une à l'autre.

3. Blanchet de caoutchouc (1) selon la revendication 1, **caractérisé en ce qu'**il comprend une couche de renforcement (4) unique en tissu, une première couche adhésive (5) pour fixer ladite couche intermédiaire (4) à ladite couche supérieure (3), et une seconde couche adhésive (6) pour fixer ladite couche intermédiaire (4) à ladite couche inférieure (2).

4. Blanchet de caoutchouc (1) selon la revendication 1, **caractérisé en ce que** ladite couche intermédiaire (4) est au moins partiellement formée à partir de tissu de coton.

5. Blanchet de caoutchouc (1) selon la revendication 1, **caractérisé en ce qu'**il consiste en une couche intermédiaire de renforcement (4) en tissu ayant une épaisseur de 0,45 mm, une première couche adhésive (5) pour fixer ladite première couche intermédiaire (4) à ladite couche supérieure (3, 3'), une seconde couche adhésive (6) pour fixer ladite couche intermédiaire (4) à ladite couche inférieure (2), une couche inférieure (2), ayant une épaisseur de 0,50 mm, et une série de couches supérieures (3, 3') ayant chacune une épaisseur de 0,35 mm.

6. Blanchet de caoutchouc (1) selon la revendication 1, **caractérisé en ce qu'**il consiste en une couche intermédiaire de renforcement (4) en tissu ayant une épaisseur de 0,45 mm, une première couche adhésive (5) pour fixer ladite première couche intermédiaire (4) à ladite couche supérieure (3), une seconde couche adhésive (6) pour fixer ladite couche intermédiaire (4) à ladite couche inférieure (2), une couche inférieure (2) ayant une épaisseur de 0,50 mm, et une couche supérieure (3) ayant une épaisseur de 0,35 mm.

7. Blanchet de caoutchouc (1) selon la revendication 1, **caractérisé en ce qu'**il consiste en une couche intermédiaire de renforcement (4) en tissu ayant une épaisseur de 0,45 mm, une première couche adhésive (5) pour fixer ladite première couche intermédiaire (4) à ladite couche supérieure (3), une seconde couche adhésive (6) pour fixer ladite couche intermédiaire (4) à ladite couche inférieure (2), une couche inférieure (2) ayant une épaisseur de 0,30 mm, et une couche supérieure (3) ayant une épaisseur de 0,55 mm.

8. Cylindre d'impression (8) sur lequel est monté le blanchet de caoutchouc (1) selon l'une quelconque des revendications précédentes, ladite surface de contact (2a) de ladite couche inférieure (2) étant directement en contact avec ledit cylindre (8) sans aucune interposition d'adhésif.
